

# UNITED STATES PATENT OFFICE.

LOUIS F. LANDA, OF FLUSHING, NEW YORK.

## POLISHING COMPOSITION.

1,278,172.

Specification of Letters Patent. Patented Sept. 10, 1918.

No Drawing.

Application filed September 20, 1917. Serial No. 192,308.

To all whom it may concern:

Be it known that I, LOUIS F. LANDA, a citizen of the United States, residing at Flushing, Long Island, in the county of 5 Queens and State of New York, have invented a certain new and useful Polishing Composition, of which the following is a specification, such as will enable those skilled in the art to which it appertains to make and 10 use the same.

The object of my invention is the production of a composition of matter for use as a polishing medium and particularly for polishing stoves and other metal articles, such 15 as radiators, steam pipes, boilers, etc.; and which may also be used for coloring, or dyeing and polishing various articles of leather such as tan shoes, belts and other articles.

My composition comprises a liquid substance, consisting of the following ingredients combined as specified;

|                      |           |
|----------------------|-----------|
| Beeswax              | 1 part.   |
| Liquid brown shellac | 19 parts. |
| Alcohol              | 22 parts. |
| Nigrosin             | 1 part.   |

In preparing my improved composition for use, the wax and shellac are first mixed and boiled, after which the alcohol is stirred 30 into the product produced by mixing and boiling the wax and shellac, and the combined product thus produced is strained and allowed to stand for an hour or so, after 35 which the nigrosin is mingled therewith by thoroughly stirring, after which the composition thus produced is bottled for use.

In polishing a stove or other metal article, the polish is applied by means of a brush and the hands are not soiled in any way, 40 and the article is given a glossy black color, which will be retained by the article to which it is applied much longer than when produced by other polishing mediums now in use. Most polishing mediums of the class 45 to which my improved composition relates

produce, when applied to metal, a dull, dark or black color, and also a disagreeable smell or odor, particularly when applied to stoves, radiators, and steam pipes, or the like, but my improved polishing composition produces a glossy black color and the use thereof 50 is not accompanied by any disagreeable smell or odor.

My improved composition may also be used for coloring, or dyeing and polishing 55 leather articles, such as tan shoes, handbags, belts and the like, and for polishing ordinary black shoes or other articles made of black leather, and for coloring or dyeing and polishing canvas shoes and other articles made of canvas, and for coloring, dyeing and polishing belts made of any material.

My invention is not limited to the exact amounts of the separate ingredients employed as herein set out, and said amounts of said ingredients may be varied within certain limits without departing from the spirit of my invention or sacrificing its advantages.

Having fully described my invention, what I claim as new and desire to secure by Letters Patent, is:

1. The composition of matter herein described, consisting of beeswax, liquid brown 75 shellac, alcohol and nigrosin combined as and for the purpose described.

2. The composition of matter herein described, consisting of beeswax 1 part; liquid brown shellac 19 parts, alcohol 22 parts 80 and nigrosin 1 part.

In testimony that I claim the foregoing as my invention I have signed my name, in presence of two subscribing witnesses, this 19th day of September, 1917.

LOUIS F. LANDA.

Witnesses:

C. E. MULREANY,  
H. E. THOMPSON.

Copies of this patent may be obtained for five cents each, by addressing the "Commissioner of Patents,  
Washington, D. C."